

## UNITED STATES PATENT OFFICE

2,383,106

WETTABLE AND DISPERSIBLE  
THIOCARBA NILIDE

Robert Ben Booth, Springdale, Conn., assignor  
to American Cyanamid Company, New York,  
N. Y., a corporation of Maine

No Drawing. Application August 10, 1944,  
Serial No. 548,931

12 Claims. (Cl. 252—61)

This invention relates to an improved dispersible thiocarbanilide.

Thiocarbanilide is an extraordinary effective froth flotation promoter, particularly for sulfide and precious metal ores. In the past, however, its use has been greatly restricted because it is very insoluble in water and is not easily wetted.

A thiocarbanilide reagent has been prepared by dissolving thiocarbanilide in dithiophosphates such as dicesyl dithiophosphoric acid, dialkyl dithiophosphoric acid and the like. Certain of these reagents have been used extensively in the froth flotation of sulfide ores. But they are subject to the limitation that only a small amount of thiocarbanilide can be dissolved, ranging from 6 to not more than 10%. Thus, the reagent is a dithio phosphate reagent and the thiocarbanilide constitutes only a minor, although important part.

D. W. Jayne (U. S. Patent No. 2,185,591) developed a new form of thiocarbanilide the individual particles of which were coated with a film of hydrophilic protective agent such as carbohydrate gums, lignin sulfonates, saponins, and the like. Preferably the particles were also coated with a powerful wetting agent such as a sulfonated alkyl naphthalene, sulfated alcohols, esters of sulfosuccinic acid, and the like. Jayne found that the thiocarbanilide treated according to his invention was effective as a sulfide reagent even though it was not soluble in the flotation pulp but was present only in a fine and uniform dispersion. The dispersible thiocarbanilide of Jayne was an immediate success. However, on extended use it was found that in the froth flotation of certain ores difficulties were encountered and it was not universally applicable.

According to the present invention, I have found that if thiocarbanilide is coated with a small amount of a sulfide promoter such as a dithiophosphate, a xanthate, a water soluble mercaptobenzothiazole and the like, the particles of thiocarbanilide disperse with the same readiness as though treated with protective colloids and wetting agents as described in the Jayne patent. At the same time no difficulty is noted from excessive foaming in the flotation cell and improved metallurgical results are obtained.

The present invention should not be confused with reagents which were prepared by dissolving a minor portion of thiocarbanilide in a major portion of dithiophosphoric acid. In the present invention the sulfide promoter such as a dithiophosphate is present as only a minor constituent normally amounting to only small percentage of

the weight of the thiocarbanilide. The effective promoter is the thiocarbanilide and the small amount of the other sulfide promoter, while probably effecting collection in a minor way, primarily tends to alter the physical characteristics of the thiocarbanilide so that it disperses readily and is thoroughly wetted.

It is important that the small amount of the sulfide promoter be admixed with the thiocarbanilide in a thorough and uniform manner so that the thiocarbanilide particles have as uniform a coating as possible. This may be effected by working the ingredients together in a thick paste in a mixer of the Werner & Pfleiderer type, by 10 milling the components together in a micropulverizer and by dry mixing in mixing equipment of the Robinson type. If desired, a small amount of a dispersing or deflocculating agent may be used to improve the uniformity of mixture and 15 may be incorporated either into the paste or dry products. These deflocculating agents include some of the products as described in the Jayne patent and also include other common dispersing or deflocculating agents such as disulfodinaphthylmethane. The purpose of dispersing or deflocculating agents in the present invention is to improve somewhat the dispersibility of the finished 20 product. The fact that improved metallurgical results are obtainable with the products of the present invention which do not contain protective colloids shows that the minor amounts of protective colloids which are present in some products do not exert any material effect in flotation.

The pastes which are obtained when the sulfide promoter and the thiocarbanilide are mixed are dispersed readily in water, and are preferred in certain flotation operations. However, many sulfide ores are located in remote parts of the world and present a serious transportation problem when pastes are used. It is, therefore, an important practical advantage of the present invention that the coated thiocarbanilide may be 40 obtained in the form of dry powder which keeps well and presents no problems of transportation. These dry powders, if properly prepared, show the same rapid and uniform dispersion possessed by the pastes. Drying of the pastes is a simple procedure requiring no difficult technique. However, the precaution should be taken to dry slowly at 45 moderate temperature, preferably in a vacuum drier, so as to prevent coagulation of any colloidal protective agents which may be present. The preparation and use of dry powders prepared as 50

described above by dry milling and mixing obviates the necessity of drying and gives uniform dispersions.

The froth flotation of sulfide ores is a very old art and has been brought to a high state of efficiency. Many ores treated are extremely low grade and the cost factor is of primary import-

5 flotation density, floated for 3 minutes in a Fagergren flotation machine. The ore was then conditioned for 3 minutes with an additional 0.1 lb./ton of the thiocarbanilide and floated for 3 minutes. 0.26 lb./ton of the pine oil was used as a frother. The results of these flotation tests are summarized in the following table.

| Thiocarbanilide used                                       | First conc.<br>percent Cu |                   | Second conc.<br>percent Cu |                   | Total Cu<br>reco.,<br>percent |
|------------------------------------------------------------|---------------------------|-------------------|----------------------------|-------------------|-------------------------------|
|                                                            | Assay                     | Distribu-<br>tion | Assay                      | Distribu-<br>tion |                               |
| Thiocarbanilide                                            | 14.76                     | 21.34             | 14.76                      | 16.21             | 37.55                         |
| Thiocarbanilide 1% sodium isopropyl naphthalene sulfonate  | 14.66                     | 15.63             | 17.76                      | 19.20             | 34.83                         |
| Thiocarbanilide 10% potassium amyl xanthate                | 18.11                     | 18.53             | 19.02                      | 20.22             | 68.75                         |
| Thiocarbanilide 5% ammonium di-sec. butyl dithiophosphate  | 25.08                     | 40.32             | 18.58                      | 50.65             | 90.97                         |
| Thiocarbanilide 8.7% sodium salts of mercaptobenzothiazole | 16.22                     | 23.68             | 14.90                      | 34.46             | 78.14                         |

tance. The improved metallurgy obtainable by the present invention, though not numerically great in the case of some ores, is of the utmost economic importance and in many cases makes a low grade ore economically amenable to beneficiation when other sulfide promoters would not permit obtaining the necessary metallurgy at low costs.

Not only does the dispersible thiocarbanilide of the present invention show improved metallurgy, but the procedure of flotation is also improved. The excessive foaming, which was definitely a problem with some ores when dispersible thiocarbanilide containing powerful wetting agents as described in the Jayne patent was used, is not present. This represents an important operating advantage.

The invention will be described in greater detail in connection with the following specific examples. The parts are by weight.

#### Example 1

A series of thiocarbanilide sulfide reagents were

20 It will be noted that the recovery with untreated thiocarbanilide and thiocarbanilide treated with a wetting agent were unsatisfactory and the grade of concentrates ranges from about 15 to under 18%. The thiocarbanilides made dispersible by the present invention show important increases in recovery with materially improved grades. Best results were obtained with the dithiophosphate and in general thiocarbanilides made dispersible by means of dithiophosphates are the preferred reagents for use in the present invention.

#### Example 2

A series of thiocarbanilides was prepared as described in Example 1, except that in addition to the sulfide reagents, a deflocculating dispersing 35 agent was included in the mixture in order to make the working easier and improve the uniformity of the product.

The procedure of Example 1, was used including the same amount of reagents.

40 The metallurgical results are summarized in the following table.

| Thiocarbanilide used                                                                                                                                                           | First conc.<br>percent Cu |                   | Second conc.<br>percent Cu |                   | Total Cu<br>reco.,<br>percent |
|--------------------------------------------------------------------------------------------------------------------------------------------------------------------------------|---------------------------|-------------------|----------------------------|-------------------|-------------------------------|
|                                                                                                                                                                                | Assay                     | Distribu-<br>tion | Assay                      | Distribu-<br>tion |                               |
| Thiocarbanilide                                                                                                                                                                | 14.76                     | 21.34             | 14.76                      | 16.21             | 37.55                         |
| Thiocarbanilide 1% sodium isopropyl naphthalene sulfonate 2% soap bark                                                                                                         | 15.70                     | 18.28             | 16.05                      | 20.53             | 38.81                         |
| Thiocarbanilide 5% potassium amyl xanthate 1% disulfodinaphthalyl-melamine                                                                                                     | 18.35                     | 35.26             | 12.67                      | 52.61             | 87.77                         |
| Thiocarbanilide 10% sodium di-sec. butyl dithiophosphate 2% of an evaporated residue from the fermentation of molasses to produce alcohol—sold in the trade under the name EMR | 22.68                     | 37.63             | 16.38                      | 52.55             | 90.18                         |
| Thiocarbanilide 4% of 1:1 mixture of sodium diethyl and di-sec. butyl dithiophosphates; 1% crude calcium lignin sulfonate                                                      | 21.10                     | 32.44             | 16.55                      | 51.45             | 83.89                         |
| Thiocarbanilide 2.5% of 1:1 mixture of sodium diethyl and di-sec. butyl dithiophosphates; 1% crude calcium lignin sulfonate                                                    | 20.83                     | 28.91             | 16.32                      | 50.15             | 79.06                         |
| Thiocarbanilide 5% ammonium di-sec. butyl dithiophosphate; 1.5% sodium lignin sulfonate                                                                                        | 20.91                     | 29.66             | 17.96                      | 58.93             | 88.59                         |
| Thiocarbanilide 8.7% sodium salt of mercaptobenzothiazole 5% crude calcium lignin sulfonate                                                                                    | 16.24                     | 15.21             | 17.44                      | 56.34             | 71.55                         |

prepared. The first was untreated; the second had incorporated 1% sodium isopropyl naphthalene sulfonate. Three other thiocarbanilides were prepared by working a paste, containing from 10 to 30% water and consisting of thiocarbanilide and 10% potassium amyl xanthate, 5% ammonium di-sec. butyl-dithio phosphate and 8.7% sodium salt of mercaptobenzothiazole respectively. The pastes were mixed thoroughly until a uniform paste was obtained. These products dispersed in water and were fed to flotation as suspensions in water.

A copper ore from the Western United States assaying about 4% copper, and containing chalcopyrite, chalcocite, covelite, enargite, pyrite, and various silicate minerals, was ground with 0.15 lb./ton of the thiocarbanilide and, after dilution to

60 65 It will be apparent that the best results are obtained by using the dispersible thiocarbanilides of the present invention. Best recoveries with high grades are obtained with the dithiophosphate modified thiocarbanilides. The poor result obtained in the second test, which is with one of the commercial reagents prepared according to the Jayne patent was due possibly to the type of froth caused by the wetting agent present in this thiocarbanilide. With many ores excellent results are obtainable with dispersible thiocarbanilide prepared according to the Jayne patent. In practically every case, however, improved metallurgy is obtained with dispersible thiocarbanilides of the present invention but the differences are not as striking as with an ore which is not practically amenable to froth flota-

tion with the Jayne thiocarbanilide. It is an advantage of the present invention that it can be used effectively with ores where the former dispersible thiocarbanilides were not practical.

*Example 3*

Tests were undertaken to determine what improvements were obtainable when thiocarbanilide is added to the flotation cell instead of to the grind as in Examples 1 and 2. The ore used was the same as in Examples 1 and 2 but was ground, diluted to flotation density, and then conditioned for 2 minutes with 0.15 lb./ton of thiocarbanilide followed by flotation in Fagergren flotation machine. The pulp was then conditioned with an additional 0.15 lb./ton of thiocarbanilide and again floated for 3 minutes; in all operations 0.026 lb./ton of pine oil was used. In the first test the dispersible thiocarbanilide of the second test of Example 2 was used, that is to say, the one worked with the isopropyl naphthalene sulfonate and soap bark. In the second test the thiocarbanilide was prepared by dry mixing the thiocarbanilide with 4% of 1:1 mixture of sodium diethyl and di-sec butyl dithiophosphates and 1% crude calcium lignin sulfonate. The metallurgical results are summarized in the following table.

| Test No. | First concentrate<br>percent Cu |                   | Second concentrate<br>percent Cu |                   | Total Cu<br>recov.,<br>percent |
|----------|---------------------------------|-------------------|----------------------------------|-------------------|--------------------------------|
|          | Assay                           | Distribu-<br>tion | Assay                            | Distribu-<br>tion |                                |
| 1.....   | 21.04                           | 20.65             | 15.84                            | 42.13             | 62.78                          |
| 2.....   | 23.40                           | 76.50             | 3.60                             | 18.57             | 95.07                          |

It will be apparent that with this procedure, a great increase in recovery and a material improvement in grade was obtained. It will be noted that the recovery was higher in the first concentrate of the second test than in both concentrates combined in the first test, that is, 76.5% as compared to about 62.8%. This accounts for the low middling product in test 2.

*Example 4*

Tests were run on a Missouri lead ore with the reagents of Example 3. The first test used the thiocarbanilide containing the isopropyl naphthalene sulfonate and soap bar while the second used that containing the dithiophosphates and lignin sulfonate. The ore contained galena, pyrite, chalcopyrite, marcasite, limestone, and quartz and assayed about 4% Pb. The ore was ground with 0.10 lb./ton thiocarbanilide added in dry form, 1.50 lb./ton trisodium phosphate and 0.25 lb./ton sodium cyanide, diluted to flotation density, and floated for 5 minutes. The resulting concentrate was cleaned by refloating for 2 minutes; 0.03 lb./ton of a higher alcohol frother, sold in the trade under the designation, B-23, was added to each of the flotation operations as a frother. The metallurgical results appear in the following table.

| Cleaner concentrate,<br>Percent Pb |              |
|------------------------------------|--------------|
| Assay                              | Distribution |
| 62.55                              | 94.16        |
| 64.64                              | 95.94        |

This example shows that even with ore for

which a dispersible thiocarbanilide of the Jayne patent is eminently suited there is still an improvement when a dispersible thiocarbanilide of the present invention is used. Both recovery and grade show increases.

When the dispersible thiocarbanilides of the present invention described in the preceding examples are prepared in paste form or by drying under vacuum or by mixing the ingredients, the products obtained show the same metallurgical results within the limits of error of ordinary flotation tests.

The following table gives the composition of a series of dispersible thiocarbanilides which can be prepared according to the present invention. In every case a product is obtained which disperses readily and which shows the improvements described in the foregoing examples.

100 parts thiocarbanilide with:

|    | As wetting agent                                                                                                                                                                                                                                                                                   | Deflocculating agent                                                                                                                                                                                                                                                                                                                                             |
|----|----------------------------------------------------------------------------------------------------------------------------------------------------------------------------------------------------------------------------------------------------------------------------------------------------|------------------------------------------------------------------------------------------------------------------------------------------------------------------------------------------------------------------------------------------------------------------------------------------------------------------------------------------------------------------|
| 20 |                                                                                                                                                                                                                                                                                                    |                                                                                                                                                                                                                                                                                                                                                                  |
| 25 | 2 to 10 parts 1:1 mixture of sodium diethyl and di-secondary butyl dithiophosphates.<br>Do.                                                                                                                                                                                                        | 0.5 to 2 parts crude calcium lignin sulfonate.<br>Do.                                                                                                                                                                                                                                                                                                            |
| 30 | 5 to 10 parts sodium di-ethyl dithiophosphate.<br>2 to 10 parts 1:1 mixture of sodium diethyl and di-secondary butyl dithiophosphates.<br>2.5 to 5 parts sodium secondary butyl xanthate.<br>2 to 5 parts sodium di-isopropyl dithiophosphate.<br>2.5 parts ammonium di-isopropyl dithiophosphate. | 1 to 2 parts sodium lignin sulfonate.<br>1 to 2 parts calcium lignin sulfonate.<br>2 parts calcium lignin sulfonate.<br>1-2 parts Tanak L (condensation product of formaldehyde and naphthalene sulfonic acid).<br>1 part calcium lignin sulfonate (crude).<br>1 to 2 parts calcium lignin sulfonate (crude).<br>1 part calcium lignin sulfonate (crude).<br>Do. |
| 35 | 5 parts ammonium di-ethyl dithiophosphate.<br>2.5 parts ammonium di-secondary butyl dithiophosphate.<br>2.5 parts sodium di-isopropyl dithiophosphate.<br>2.5 parts 1:1 mixture of sodium salts of mercaptobenzothiazole and di-secondary butyl dithiophosphoric acid.                             | 1 part Tanak L calcium lignin sulfonate (crude).<br>1 part calcium lignin sulfonate (crude).<br>Do.                                                                                                                                                                                                                                                              |
| 40 | 5 parts sodium salt of mercaptobenzothiazole.<br>2.5 to 5 parts sodium secondary butyl xanthate.<br>2.5 parts sodium ethyl xanthate.                                                                                                                                                               | 1 part Tanak L.                                                                                                                                                                                                                                                                                                                                                  |
| 45 | 2.5 parts potassium isopropyl xanthate.<br>2.5 parts potassium amyl xanthate.<br>2.5 parts 1:1 mixture of sodium diethyl and di-secondary butyl dithiophosphate.                                                                                                                                   | Do.<br>Do.<br>Do.                                                                                                                                                                                                                                                                                                                                                |
| 50 | Do.<br>Do.<br>2 to 5 parts sodium di-isopropyl dithiophosphate.<br>Do.                                                                                                                                                                                                                             | 1 part calcium lignin sulfonate (crude).<br>1 part Tanak A (condensation product of formaldehyde and naphthalene sulfonic acid).<br>1 part Sap Brown.<br>1 part E.M.E.<br>1 part nigrosine (water-soluble).<br>1 part yellow corn dextrine.                                                                                                                      |
| 55 | Do.<br>Do.<br>2.5 parts sodium di-secondary butyl dithiophosphate.                                                                                                                                                                                                                                 | 1 part sodium lignin sulfonate.<br>1 part calcium lignin sulfonate.<br>1 part Blanco (condensation product of formaldehyde and naphthalene sulfonic acid).                                                                                                                                                                                                       |

60 As in the examples there will be differences in the effectiveness of the various products. The most economical reagent is in the first line of the table, as it combines high efficiency with low cost. The above products are equally useful as pastes and as dry powders where the drying is effected carefully so as to prevent any irreversible change in the deflocculating agent or the dry product is prepared by thorough mixing of the dry ingredients.

I claim:

70 1. A dispersible thiocarbanilide comprising thiocarbanilide the individual particles of which are coated with a film of a sulfide promoter selected in the group consisting of organic esters of dithiophosphoric acid, xanthates and water soluble mercaptobenzothiazoles, the sulfide promoter being present in a minor proportion in

comparison to the thiocarbanilide and the coating being sufficiently uniform to produce a product which is readily dispersible in water and in the pulp in froth flotation operations.

2. A free flowing dispersible thiocarbanilide promoter in which the individual particles of which are coated with a film of sulfide promoter selected in the group consisting of organic esters of dithiophosphoric acid, xanthates and water soluble mercaptobenzothiazoles, the sulfide promoter being present in a minor proportion in comparison to the thiocarbanilide and the coating being sufficiently uniform to produce a product which is readily dispersible in water and in the pulp in froth flotation operations.

3. A dispersible thiocarbanilide according to claim 1 in which the sulfide promoter is a dithiophosphate.

4. A dispersible thiocarbanilide according to claim 2 in which the sulfide promoter is a dithiophosphate.

5. A dispersible thiocarbanilide according to claim 1 in which the sulfide promoter is a xanthate.

6. A dispersible thiocarbanilide according to claim 2 in which the sulfide promoter is a xanthate.

7. A dispersible thiocarbanilide according to claim 1 in which the sulfide promoter is a water soluble mercaptobenzothiazole.

8. A dispersible thiocarbanilide according to claim 2 in which the sulfide promoter is a water soluble mercaptobenzothiazole.

9. A dispersible thiocarbanilide according to claim 1 in which the coating of the thiocarbanilide particles includes a minor portion of a deflocculating agent.

10. A dispersible thiocarbanilide according to claim 2 in which the coating of the thiocarbanilide particles includes a minor portion of a deflocculating agent.

15. 11. A dispersible thiocarbanilide according to claim 1 in which the coating of the thiocarbanilide particles contains a mixture of dialkyl-dithiophosphates and at least one lignin sulfonate.

20. 12. A dispersible thiocarbanilide according to claim 2 in which the coating of the thiocarbanilide particles contains a mixture of dialkyl-dithiophosphates and at least one lignin sulfonate.

ROBERT BEN BOOTH.